

## UNITED STATES PATENT OFFICE

MAX BOMMER AND ROBERT HALLER, OF RIEHEN, NEAR BASEL, SWITZERLAND, AND ENRICO POOL, OF BASEL, SWITZERLAND, ASSIGNORS TO FIRM SOCIETY OF CHEMICAL INDUSTRY IN BASLE, OF BASEL, SWITZERLAND

## PROCESS FOR OBTAINING FAST TINTS ON THE FIBER

No Drawing. Application filed December 16, 1931, Serial No. 581,514, and in Switzerland January 15, 1931.

In U. S. patent application Serial No. 389,324, filed August 29, 1929, it has been shown that leuco-derivatives of vat-dyestuffs react with diazo-compounds on the fiber to produce colored pigments. These pigments color the fiber fast tints which are quite different from those that are obtained with the vat-dyestuffs alone.

The further study of this reaction has led to the present invention, namely a process wherein fibers, which have been dyed with vat-dyestuffs that must in practice be vatted with the aid of hydrosulfite, are treated with diazo-compounds.

It was found that the dyeings produced with the vat-dyestuffs enter into reaction with the diazo-compounds.

In this manner tints are obtained which are more or less strongly different from the dyeings of the untreated vat-dyestuff and are distinguished from the latter in many cases by their intensity and enhanced fastness.

The process is applicable with very different vat-dyestuffs which in practice must be vatted with the aid of hydrosulfite; such are, for instance, the anthraquinone vat-dyestuffs, the indigoid vat-dyestuffs and the products of sulfurization of carbazole-indophenols.

The new process is particularly valuable when the products of sulfurization of carbazole indophenols are used as the vat-dyestuffs and diazotized aminoazo-dyestuffs are used as the diazo-compounds, because in these cases there are obtained as a rule dyeings of black shade and, at the same time, of remarkable fastness.

The invention can be applied for obtaining fast tints on all fibers which can be dyed with vat-dyestuffs. For instance, cotton, wool, loaded or unloaded silk, artificial fibrous material of all kinds.

The following examples illustrate the invention:—

## Example 1

A 10 per cent. dyeing of Hydron Blue R (Schultz, 7th Edition, No. 1111) is treated for  $\frac{1}{2}$  hour at room temperature in a bath containing an excess of sodium acetate and

8 grams per litre of 4'-chloro-2-methyl-5-methoxy-4-diazo-azobenzene. The material is then rinsed, acidified, again rinsed, and dried. The blue dyeing passes into a deep, fast black, particularly fast to kier boiling. 55

The substitution of other diazotized amino-azo-compounds, for instance diazotized benzeneazo- $\alpha$ -naphthyl-amine for the 4'-chloro-2-methyl-5-methoxy-4-diazo-azobenzene used in this example, produces as a rule 60 similar black dyeings.

Dark marine blue tints are obtainable with the tetrazotized aminoazo-compound from 4'-amino-2-methyl-5-methoxy-4-amino-azo-benzene and with more simple diazo-compounds, such as diazotized 2:5-dichloraniline, 5-nitro-ortho-anisidine, meta-nitro-para-toluidine, meta-chloraniline, 4-chloro-ortho-nitraniline, 4-chloro-2-amino-1:1'-di-phenyl-ether. 65

Instead of the Hydron Blue R there may be used, for example, Hydron Blue G (Schultz, 7th Edition, No. 1113).

## Example 2

A 5 per cent. dyeing of Ciba Red R (Schultz, 7th Edition, No. 1339) is treated for  $\frac{1}{2}$  hour at room temperature in a bath containing an excess of sodium acetate and 8 grams per litre of diazotized 4-chloro-2-nitraniline. The material is then rinsed, acidified, again rinsed, and dried. The red dyeing becomes fuller and more yellow. 75

If one treats in similar manner a 2.5 per cent. dyeing of Ciba Red 3B (Schultz, 7th Edition, No. 1354) with 4'-chloro-2-methyl-5-methoxy-4-diazo-azobenzene, the red-violet dyeing passes into an intense, pure, yellowish bordeaux, which is characterized by a very good fastness to kier boiling. 80 85 90

## Example 3

A 2.5 per cent. dyeing of Cibanone Blue RS (Schultz, 7th Edition, No. 1228) is treated for  $\frac{1}{2}$  hour at room temperature in a bath containing an excess of sodium acetate and 8 grams per litre of 4'-chloro-2-methyl-5-methoxy-4-diazo-azobenzene; the blue dyeing passes into grey. The material is then rinsed, acidified, again rinsed, and dried. By 100

substituting for the diazotized aminoazo-dyestuff diazotized 4-chloro-ortho-nitraniline, a very greenish grey is obtained.

A similar procedure may be adopted with other dyestuffs of the anthraquinone series or of the benzanthrone, pyranthrone, anthranthrone, dibenzpyrenequinone and the like series.

For example, with Cibanon Gold Orange 10 GN (Schultz, 7th Edition, No. 1245) and 4'-chloro-2-methyl-5-methoxy-4-diazo-azobenzene there is a change from orange to brown.

What we claim is:—

1. Process for obtaining fast tints on the fiber, which consists in causing dyeings which have been produced with such vat-dyestuffs that must in practice be vatted with the aid of hydrosulfite to react with diazo-compounds.
2. Process for obtaining fast tints on the fiber, which consists in causing dyeings which have been produced with anthraquinone vat-dyestuffs to react with diazo-compounds.
3. Process for obtaining fast tints on the fiber, which consists in causing dyeings which have been produced with indigoid vat-dyestuffs to react with diazo-compounds.
4. Process for obtaining fast tints on the fiber, which consists in causing dyeings which have been produced with the products of sulfurization of carbazole-indophenols to react with diazo-compounds.
5. Process for obtaining fast tints on the fiber, which consists in causing dyeings which have been produced with the products of sulfurization of carbazole-indophenols to react with diazotized aminoazo dyestuffs.

In witness whereof we have hereunto signed our names this 7th day of December 1931.

MAX BOMMER.  
ROBERT HALLER.  
ENRICO POOL.

45

50

55

60

65